

June 2, 1942.

J. DUSEVOIR

2,284,729

METHOD OF CASTING FINNED CYLINDER HEADS

Filed Oct. 6, 1941



INVENTOR

Julius Dusevoir.  
BY  
Harness, Dickey & Pierce.  
ATTORNEYS.

## UNITED STATES PATENT OFFICE

2,284,729

## METHOD OF CASTING FINNED CYLINDER HEADS

Julius Dusevoir, Dearborn, Mich., assignor to  
 Century Motors Corporation, Dearborn, Mich.,  
 a corporation of Michigan

Application October 6, 1941, Serial No. 413,739

16 Claims. (Cl. 22—126)

This invention relates to the casting of finned cylinder heads for internal combustion engines of the air cooled type and has for its principal object the provision of such method by the practice of which more perfect castings may be obtained than heretofore possible, as well as to a mold for use in connection therewith.

Objects of the invention include a method of casting a finned cylinder head comprising forming a mold part for the finned portion of the head from a refractory heat insulating material and forming another mold part for the combustion chamber portion of the head from a heat conducting material, casting the molten metal into the mold and circulating a cooling medium in contact with the heat conducting portion of the mold before the metal has had an opportunity to completely set, whereby to accelerate the cooling of that portion of the metal defining the combustion chamber of the head; the provision of a method as above described in which the fin forming portion of the mold is formed principally from sand; the provision of a method as above described in which that portion of the mold defining the combustion chamber of the head is formed from metal and provided with hollow walls through which a cooling medium is circulated; and the provision of a method as above described in which the heat conducting portion of the mold is heated prior to the placing of the molten metal in the mold and is cooled intermediate the time the molten metal is poured and is completely solidified.

Other objects of the invention include the provision of a mold for casting finned cylinder heads for internal combustion engines of the air cooled type for non-hardening metal comprising a mold portion for forming the finned surface of the cylinder head presenting a refractory surface of low heat conductivity for contact with the molten metal poured into the mold, and a mold portion for forming the combustion chamber portion of the head including a bare metal surface for contact with the molten metal; the provision of a mold as above described having means for heating the bare metal surface preliminary to the casting operation; the provision of a mold as above described having means for cooling the bare metal surface; the provision of a mold as above described having means for first heating and then cooling the bare metal surface; the provision of a mold as above described in which the bare metal portion forms a part of a metallic mold part having hollow walls through which a heat exchange medium is adapted to be cir-

culated; and the provision of a mold as above described that is capable of yielding under the contracting pressure of the surrounding casting during cooling thereof.

The above being among the objects of the present invention the same consists in certain novel features of construction, combination of parts and steps of operation to be hereinafter described with reference to the accompanying drawing, and then claimed, having the above and other objects in view.

In the accompanying drawing which illustrates a suitable embodiment of a cylinder head and of apparatus which may be employed in the casting of the same in accordance with the present invention, and in which like numerals refer to like parts in both the views,

Fig. 1 is a fragmentary side elevational view of a cylinder for an internal combustion engine of the air cooled type illustrating the same as being provided with a finned cylinder head;

Fig. 2 is a more or less diagrammatic vertical sectional view taken centrally through a mold employed for casting the cylinder head shown in Fig. 1, and

Fig. 3 is a top plan view of the metallic insert for the mold shown in Fig. 2.

As is commonly understood the cylinder heads for air cooled engines are cast with cooling fins formed integrally therewith and the under side of the heads commonly form the combustion chamber for the associated cylinders. The main portion of such head which forms the combustion chamber and forms a means for connecting the head to the cylinder must be relatively heavy in order to withstand the explosion pressures occurring within the combustion chamber and to permit the head to be secured to the cylinder with required security and sealing effect. On the other hand the fins, in order to be as efficient as possible in the dissipation of heat from the head to the surrounding air, must be relatively thin. As a result of the relatively thick body and the relatively thin fins, regardless of the metal employed, certain foundry problems arise in the casting of such heads due to unequal cooling and, therefore, unequal shrinkage of the metal in changing from the molten to the solid state. Aluminum is the metal most commonly used in forming such cylinder heads and its coefficient of contraction in solidifying is higher than most metals, thus causing the above described problems to be present to a greater extent. For this reason reference herein will, for the purpose of simplicity in explanation, be limited to the ex-

planation of the present invention in connection with casting of aluminum cylinder heads only, it being understood that the problems involved and the method of overcoming them are likewise applicable to the casting of such heads from other metals and particularly those light metals or alloys thereof having a relatively high coefficient of contraction when changing from the molten to the solid state.

From the standpoint of foundry practice, if unequal sections of metal are cast in one piece in accordance with conventional practice, heat is dissipated from the thin sectioned part faster than the other, causing such thin part to solidify before the thicker part and in solidifying to pull some of the molten metal away from the thicker part, thus causing shrinkages which cause a change in the grain of the metal, gas holes, core disturbances and other defects which make such a problem a serious one in the foundry. Particularly where such parts being cast are cylinder heads of the type above described and are formed from aluminum or other light metal having a high coefficient of contraction when changing from the liquid to the solid state the problem becomes so serious that a material percentage of the castings have to be scrapped when cast in accordance with conventional practices. Fine cracks or checks appear in the surface of the combustion chamber side of the head which appear to be caused by cracks in the sand core. Inasmuch as the combustion chamber surface of the head is required to be of solid metal free from all defects, the presence of such cracks or checks form defects which require the scrapping of many of such castings. Heretofore in attempting to overcome such defects in cylinder heads cast in accordance with conventional practice the combustion chamber side of the casting has been thickened and the excess metal machined away in an endeavor to cut away the checked surface and present clean solid metal in the final product. However, it has been my experience that such procedure only aggravates the conditions initially forming such checks or other imperfections in that it still further aggravates the difference in thickness between the main portion of the head and the fins, besides involving a material amount of additional cost in the excessive machining operations necessarily resulting to bring the head to its finished condition.

The present invention, which is designed to overcome the defects above described resulting from conventional methods of casting such cylinder heads, is based upon the assumption that if the thicker portion of the head can be cooled at a rate more nearly commensurate with the rate of cooling of the fins themselves, or at least at a rate sufficient to cause the metal for such thickened portion to solidify simultaneously with solidification of the metal for the fins, it will eliminate the withdrawal by the fins of heat from the thickened portion of the head which now occurs in the practice of the conventional casting methods. Such withdrawal of heat from the thickened portion will occur at a time when, in the practice of conventional methods, the metal in the fins is solidified and the metal in the thicker portion of the head still remains in molten or partially molten condition. It is, therefore, based upon the assumption that if in the casting operation this withdrawal of the heat by the fins from the thick portion of the head can be stopped completely, or to a major extent,

the effects thereof on the casting can be eliminated and the defects occurring in such castings cast in accordance with the conventional methods eliminated. Practice has proven that these assumptions are correct.

In order to withdraw heat from the thick portion of the head and particularly from that surface thereof forming the combustion chamber means other than the usual sand core must be employed. In accordance with the present invention that surface of the mold forming the combustion chamber side of the head is formed from a heat conducting material, or more specifically from metal, and after the pouring operation is completed this metal is quickly cooled so as to abstract heat from the combustion chamber side of the thick metal portion of the head. This cooling may be accomplished in the broader aspects of the invention in any suitable way, but in order to abstract the heat as fast as possible it is preferable to circulate a cold fluid and preferably a cold brine in contact therewith. For this purpose the metallic part of the mold is preferably made with hollow walls through which such brine or other suitable cooling fluid may be circulated with desired effectiveness and speed and such metal surface is allowed to remain bare or at least substantially devoid of any heat insulating material. It is important to note that such metal portion is not used as a chill in the ordinary sense in that no attempt is made to harden the metal coming in contact with it, this being impossible because of the character of the metal being cast. Its purpose is solely to cause solidification of the metal for the thick portion of the casting at a rate commensurate with the solidification of the metal for the fins.

Where the shape of the combustion chamber is such that the metallic part of the mold is substantially surrounded by the molten metal during the casting operation, then with certain designs of combustion chambers and particularly in the larger sizes, unless some provisions are made to remedy it, the cast metal in solidifying and cooling may shrink to such an extent about the unyielding metallic part of the mold as to actually cause portions of the casting to be split. To overcome this difficulty, in a more limited sense the present invention provides a construction which will permit the metal portion of the mold thus surrounded by the casting being made to yield under the contracting pressure of the cooling casting so as to minimize the strains thus set up in the casting. This is preferably accomplished by slotting or otherwise forming the metal portion so as to provide a plurality of parts or segments yieldably connected together.

Referring now to the accompanying drawing and particularly to Fig. 1 a cylinder head is shown which may be assumed to be representative of the general class of cylinder heads under discussion and which take a multitude of different shapes, sizes and contours in different makes of engines. In Fig. 1 the cylinder is indicated at 10 and as having a plurality of peripheral annular fins 12 formed thereon. The upper end of the cylinder 10 is provided with a relatively heavy flange 14 through which the cylinder head is adapted to be secured to the cylinder. The cylinder head includes a relatively heavy main flanged edge 15 and body portion 16 of substantially the same thickness provided with a pair of hollow bosses 18 serving as inlet and outlet ports

for the associated cylinder. Fins 20 are formed integrally with the main body portion 16 and bosses 18. As indicated in Fig. 2 the cylinder head is interiorly formed to provide a combustion chamber space 22, and while this may be of any desired size, shape and contour, as a matter of illustration it is shown in the present case as being partially spherical.

Referring now to Fig. 2 the mold for forming the cylinder head shown in Fig. 1 is illustrated, the mold cavity being shown filled with metal in the condition it assumes after the pouring operation. It will be understood that the showing in Fig. 2 is more or less diagrammatic particularly in view of the fact that it will be appreciated that in connection with the particular cylinder head shown the cope will ordinarily have to be formed in separate parts to permit the removal of the pattern in view of the differently directed fins 20 in the final product. In any event, however, the mold will include a drag 30 and cope 32. Depending upon the particular foundry practice followed, the cope 32 may be green sand or it may be of baked sand such as is conventionally employed for forming cores; and the cavity therein is complementary in shape to the exterior surfaces of the cylinder head with the exception that two cores 34 are mounted therein for forming the hollow interior of the bosses 18. On the other hand the cope 32 may be of a permanent character such as is conventionally employed in so-called permanent molds. That is, it may be made up of one or more metallic parts in which case the surfaces forming the mold cavity therein will be coated with a suitable thickness of refractory material to insulate it against too rapid an absorption of heat from the molten metal cast therein. In any event and regardless of the construction of the cope 32 it will, of course, be appreciated that it will be provided with a sprue hole 36 and a gate 38 connecting the sprue hole 36 with some suitable part of the cavity therein as for instance that portion thereof in which the flange 15 is formed and as indicated.

The drag 30 may be of any suitable character and construction as long as it incorporates the features of the present invention. In other words, it may be of a permanent character as above described, it may be formed of green sand with the metallic combustion chamber forming portion hereinafter described included as an insertion therein, or it may be formed of baked sand with such insertion therein. For the purpose of illustration it may be assumed in the case shown that the drag 30 includes a main body portion 40 formed from baked sand and formed about an insert indicated generally at 42 which is imbedded in the main body portion 40. The insert 42 is formed from metal and while the particular metal employed for this purpose is more or less unimportant as long as its melting point temperature is not such that the molten metal introduced into the mold cavities will tend to fuse thereto, where the cylinder head being cast is to be formed from aluminum it may be conveniently formed from cast iron. The upper surface of the insert 42 is formed as a part of a spherical surface in the particular case shown and complementary at least in part to the size and shape of the combustion chamber cavity 22 desired in the cylinder head, due allowance, of course, being made for shrinkage during the solidifying of the metal in the mold and machining stock where desired. In other words, the

upper portion of the insert 42 is complementary in size, shape and contour, with required allowances for contraction of the metal and machining stock where desired, to the combustion cavity 22. In the particular case shown the partially spherical upper surface of the insert 42 is extended downwardly into the main portion 40 of the drag 30 and is there reduced to form a cylindrical collar 44. In the particular case shown the insert 42 not only is hollow but it is provided with hollow walls forming a passage 46 therein for the circulation of heating and/or cooling mediums therethrough. Such heating and/or cooling medium may be introduced into the passage 46 in any suitable manner as, for instance, by means of a pipe 48 extending up through the hollow interior of the insert 42 and threaded through one-half of the hollow wall thereof so as to discharge its contents centrally of the hollow walls of the insert. Such heating and/or cooling medium may be discharged from such hollow walls by means of one or more discharge pipes 50 which, in the particular case shown, are threaded into the lower edge of the collar 44 and into communication with the passage 46 therein.

In the particular construction shown, because of the fact that the insert 42 is substantially semi-spherical it is possible that difficulty might arise due to the shrinkage of the metal in cooling during the cooling of the casting about it. In other words if the insert 42 was solid and unyielding it would present an uncompressible part about which the molten metal would attempt to shrink, and this occurring at a time when the metal of the casting is at an elevated temperature and, therefore, of low tensile strength might cause the casting to be split under the shrinkage strains. Where such a condition exists it is preferable to so design the insert as to render it capable of yielding under this contracting pressure in order to prevent the possibility above mentioned. This is preferably accomplished by forming the insert as a plurality of yieldably connected parts capable of yielding under the contracting pressure of the casting during shrinkage. In the particular case shown this is accomplished by forming four slots 60 in the insert 42, such slots being located in two planes perpendicular to each other and with their line of intersection coincident with the axis of the insert 42. These slots extend from the lower edge of the insert 42 to a point adjacent to but spaced from the center of the insert 42 at its upper end, as shown, to thus provide four equally angularly disposed segments connected to each other over a limited area at the top of the insert. The slots 60 do not, of course, cut into the passages 46 but are suitably walled off therefrom as indicated in Fig. 3 so that the passage in one segment is connected to the passages in the remaining segments only at the center of the insert. A discharge pipe 50 is, of course, connected into the passage 46 for each segment.

The slots 60 are preferably filled with green molding sand or some other resilient or yieldable material to prevent the molten metal from escaping through them. Such material should be capable of yielding or being displaced under the pressure which is exerted upon it when the segments of the insert are squeezed toward each other as the metal contracts about the insert and, of course, resistant to the heat of the molten metal. On the upper face of the insert 42 the material filling the slots 60 is brought into flush

relationship with the adjacent faces of the insert so as to present a smooth, unbroken surface. Thus where green sand, for instance, is employed to fill the slots 60 for a casting operation, when the casting contracts about the insert the various segments will yield inwardly about their areas of connection with the central portion of the insert, the green sand in the slots 60 simply being squeezed out into the center of the insert under the contracting force applied to the insert.

It will be understood that the exposed surface of insert 42 in the mold is not covered by any refractory material which would materially reduce its heat absorbing capacity when in contact with the molten metal, but at the most it will be merely given a light coating of lamp black or other dry lubricant to prevent possibility of the molten metal sticking to its surface.

In some cases it may be satisfactory to pour the molten metal into the mold without pre-heating the insert 42 and before cooling of the same has been started, but in most instances it will be preferable if the insert 42 is heated immediately prior to the pouring operation so as not to materially chill the molten metal coming in contact with it before the mold has had an opportunity to become completely filled with molten metal. Where such preliminary heating is desired the same circulating passage employed for circulating the cooling fluid may be employed for circulating a heating medium. In such case the pipe 48 may be provided with a three-way valve 52 to which is connected a pipe 54 connected to a suitable source of cooling medium under pressure and a pipe 56 connected to a suitable source of heating medium under pressure. The source of cooling medium to which the pipe 54 may be connected may be suitably cooled air or other gaseous medium or may be a suitably cooled liquid medium. Preferably a cold brine under pressure is employed as a cooling medium. Likewise the pipe 56 may be connected to any suitable source of heating medium and while this may be either in a gaseous or liquid form it is preferably in a gaseous form, as for instance highly heated air, so that there will be no problem in the separation of the heating and cooling mediums which may momentarily intermingle upon shifting of the valve 52, this being particularly desirable where one of such mediums is to be re-circulated.

Where no preliminary heating of the insert 42 is to be done, the valve connecting the pipe 48 with a source of cooling medium is closed, a suitable charge of molten metal is poured into the sprue hole 36 to charge the mold until the mold is completely filled, the metal is allowed to partially set or solidify and then the valve is turned on to cause a rush of the cooling fluid through the hollow walls of the insert, thus withdrawing heat from the combustion chamber surface portion 22 of the casting and accelerating the solidification of the metal therearound. The metal forming the fins 20 being relatively thin in section and having an extended surface in contact with the material of the cope 32, of course solidifies much faster than the metal in the main body portion 16 of the cylinder head under ordinary circumstances, and in cooling and contracting draws in metal from the main body portion 16 when cast according to conventional practices with the resulting disadvantages previously explained, that is the formation of cracks, blow holes, and the like particularly in the sur-

face 22 of the cylinder head. By employing an insert such as 42 of relatively high heat conducting capacity and forcing a cooling medium through the hollow walls thereof, the metal of the main body portion 16 is caused to solidify at a rate commensurate with the rate of solidification of the metal in the fins 20, the result being that the casting is solidified more or less uniformly throughout during its transition from the molten to the solid state. Tests have indicated that by following out the above described procedure the defects occurring in cylinder heads of the type described cast in accordance with conventional methods are substantially entirely eliminated, and the percentage of scrap heads resulting from casting in accordance with the present invention is a fraction only of the heads scrapped because of defects occurring when cast by conventional methods.

Where cylinder heads cast as above described indicate freezing of the metal in contact with the insert 42 prior to complete filling of the mold, then preliminary heating of the insert 42 may be resorted to by means of introducing a suitable heating medium through the pipe 56 and then through the pipe 48 to the hollow walls of the insert 42. In such case the heating medium is, of course, introduced into the insert 42 before the metal is poured and may be discontinued immediately prior to the pouring operation, immediately upon completion of the pouring operation, or may be discontinued the moment before circulation of the cooling medium is commenced. In any event it will be understood that under such circumstances when the metal is poured into the mold the insert 42 is raised in temperature sufficiently to obviate any possible or at least detrimental freezing of the metal in contact with the insert 42 prior to completing the pouring of the mold, and that in any case after the molten metal has been given an opportunity to partially set, the valve 52 is turned to cause an immediate forced circulation of the cooling medium through the insert thereby to quickly abstract the heat from the surface 22 of the casting.

Having thus described my invention what I claim by Letters Patent is:

1. The method of forming a cast light metal cylinder head having a relatively thick body provided with a multiplicity of relatively thin cooling fins on one side thereof and formed to provide a combustion chamber cavity on the opposite side thereof, comprising the steps of casting molten metal to substantially the size, shape and contour of said head, protecting said finned side of said molten metal casting against rapid loss of heat from the surface thereof, and only after said molten metal has partially set but is still in partially molten condition rapidly withdrawing heat from said opposite side thereof.

2. The method of forming a cast light metal cylinder head having a relatively thick body provided with a multiplicity of relatively thin cooling fins on one side thereof and formed to provide a combustion chamber cavity on the opposite side thereof, comprising the steps of casting molten metal to substantially the size, shape and contour of said head, protecting said finned side of said molten metal casting against rapid loss of heat from the surface thereof, and only after said molten metal has partially set but is still in partially molten condition rapidly withdrawing heat from said opposite side thereof by the circulation of a cooling medium in heat con-

ducting relation with respect thereto, whereby to effect approximately uniform solidification of said molten metal throughout said casting.

3. The method of forming a cast light metal cylinder head having a relatively thick body provided with a multiplicity of relatively thin cooling fins on one side thereof and formed to provide a combustion chamber cavity on the opposite side thereof, comprising the steps of casting molten metal to substantially the size, shape and contour of said head, protecting said finned side of said molten metal casting against rapid loss of heat from the surface thereof, delaying solidification of said molten metal on said opposite side by retarding the loss of heat therefrom until a part only of said molten metal has solidified, and then rapidly withdrawing heat from said opposite side commencing while said molten metal is in partly molten condition to accelerate the solidification of said molten metal on said opposite side.

4. The method of forming a cast light metal cylinder head having a relatively thick body provided with a multiplicity of relatively thin cooling fins on one side thereof and formed to provide a combustion chamber cavity on the opposite side thereof, comprising the steps of casting molten metal to substantially the size, shape and contour of said head, protecting said finned side of said molten metal casting against rapid loss of heat from the surface thereof, delaying solidification of said molten metal on said opposite side by retarding the loss of heat therefrom until a part only of said molten metal has solidified, and then rapidly withdrawing heat from said opposite side commencing while said molten metal is in partly molten condition by the forced circulation of a cooling medium in metallic heat conducting relation with respect thereto to accelerate the solidification of said molten metal on said opposite side.

5. The method of forming a cast light metal cylinder head having a relatively thick body provided with a multiplicity of relatively thin cooling fins on one surface thereof and formed to present a combustion chamber cavity on the other side thereof comprising, in combination, forming a mold with a cavity substantially complementary in size, shape and contour to the desired cast head and with that surface complementary to said surface having said fins of a refractory material and that surface complementary to said combustion chamber cavity of substantially bare metal, filling said mold cavity with molten metal, and effecting a circulation of cooling medium in heat conducting relation with respect to said bare metal surface commencing at a time after said mold has been filled by said molten metal and before said molten metal has completely solidified in said mold cavity.

6. The method of casting a cylinder head having a multiplicity of relatively thin external cooling fins and a combustion chamber cavity on the side thereof opposite said fins, comprising the steps of forming a mold having a cavity complementary to said cylinder head and with that surface of said mold cavity complementary to said finned surface of said cylinder head formed of a refractory material of low heat conductivity and that surface of said mold cavity complementary to said combustion chamber cavity of substantially uninsulated metal, filling said mold cavity with molten metal, and abstracting heat from said metal surface of said mold cavity by the circulation of a cooling fluid in heat con-

ducting relation therewith after said mold cavity has been filled with said molten metal but beginning at a time before said molten metal in said mold cavity has become completely solidified.

5. 7. A mold for forming a cast light metal cylinder head having a relatively thick body portion provided with a multiplicity of relatively thin cooling fins projecting outwardly from one side thereof and formed to present a combustion chamber cavity on the opposite side thereof comprising, in combination, a mold portion presenting a refractory surface complementary in size, shape and contour to said finned side of said head, and a mold portion presenting an uninsulated surface of bare metal complementary in size, shape and contour to said combustion chamber cavity, said uninsulated metal surface being arranged in metallic heat conducting relationship with respect to a fluid circulation passage.

10 8. A mold for forming a cast light metal cylinder head having a relatively thick body portion provided with a multiplicity of relatively thin cooling fins projecting outwardly from one side thereof and formed to present a combustion chamber cavity on the opposite side thereof comprising, in combination, a mold portion presenting a refractory surface complementary in size, shape and contour to said finned side of said head, and a mold portion presenting an uninsulated surface of bare metal complementary in size, shape and contour to said combustion chamber cavity, said uninsulated metal surface comprising a part of a hollow walled element the walls of which are provided with a fluid circulation inlet and outlet passage.

15 9. A mold for forming a cast light metal cylinder head having a relatively thick body portion provided with a multiplicity of relatively thin cooling fins projecting outwardly from one side thereof and formed to present a combustion chamber cavity on the opposite side thereof comprising, in combination, a mold portion presenting a refractory surface complementary in size, shape and contour to said finned side of said head, and a metallic, hollow walled mold portion presenting a substantially bare metal surface complementary in size, shape and contour to said combustion chamber cavity.

20 10. A mold for forming a cast light metal cylinder head having a relatively thick body portion provided with a multiplicity of relatively thin cooling fins projecting outwardly from one side thereof and formed to present a combustion chamber cavity on the opposite side thereof comprising, in combination, a mold portion presenting a refractory surface complementary in size, shape and contour to said finned side of said head, a metallic, hollow walled mold portion presenting a substantially bare metal surface complementary in size, shape and contour to said combustion chamber cavity, and means for circulating a heating medium through said hollow walls.

25 11. A mold for forming a cast light metal cylinder head having a relatively thick body portion provided with a multiplicity of relatively thin cooling fins projecting outwardly from one side thereof and formed to present a combustion chamber cavity on the opposite side thereof comprising, in combination, a mold portion presenting a refractory surface complementary in size, shape and contour to said finned side of said head, a metallic, hollow walled mold portion presenting a substantially bare metal surface complementary in size, shape and contour to said

combustion chamber cavity, and means for circulating a cooling medium through said hollow walls.

12. A mold for forming a cast light metal cylinder head having a relatively thick body portion provided with a multiplicity of relatively thin cooling fins projecting outwardly from one side thereof and formed to present a combustion chamber cavity on the opposite side thereof comprising, in combination, a mold portion presenting a refractory surface complementary in size, shape and contour to said finned side of said head, a metallic, hollow walled mold portion presenting a substantially bare metal surface complementary in size, shape and contour to said combustion chamber cavity, means for circulating a heating medium through said hollow walls, and means for circulating a cooling medium through said hollow walls.

13. A mold for forming a cast light metal cylinder head having a relatively thick body portion provided with a multiplicity of relatively thin cooling fins projecting outwardly from one side thereof and formed to present a combustion chamber cavity on the opposite side thereof comprising, in combination, a mold portion presenting a refractory surface complementary in size, shape and contour to said finned side of said head, a metallic, hollow walled mold portion presenting a substantially bare metal surface complementary in size, shape and contour to said combustion chamber cavity, means for circulating a heating medium through said hollow walls, means for circulating a cooling medium through said hollow walls, and control means for said mediums operable to permit flow of one of said mediums only at one time through said hollow walls.

14. A mold for forming a cast light metal cylinder head having a relatively thick body portion provided with a multiplicity of relatively thin cooling fins projecting outwardly from one side thereof and formed to present a combustion chamber cavity on the opposite side thereof comprising, in combination, a mold portion presenting a refractory surface complementary in size, shape and contour to said finned side of said head, and a contractible mold portion pre-

senting an uninsulated surface of bare metal complementary in size, shape and contour to said combustion chamber cavity, said uninsulated metal surface being arranged in metallic heat conducting relationship with respect to a fluid circulation passage.

15. A mold for forming a cast light metal cylinder head having a relatively thick body portion provided with a multiplicity of relatively thin cooling fins projecting outwardly from one side thereof and formed to present a combustion chamber cavity on the opposite side thereof comprising, in combination, a mold portion presenting a refractory surface complementary in size, shape and contour to said finned side of said head, and a mold portion presenting an uninsulated surface of bare metal complementary in size, shape and contour to said combustion chamber cavity, said uninsulated metal surface comprising a part of a hollow walled element the walls of which are provided with a fluid circulation inlet and outlet passage and including a plurality of portions each directly fixed to the next adjacent thereof but yieldable with respect to one another under the influence of metal contracting thereabout.

16. A mold for forming a cast light metal cylinder head having a relatively thick body portion provided with a multiplicity of relatively thin cooling fins projecting outwardly from one side thereof and formed to present a combustion chamber cavity on the opposite side thereof comprising, in combination, a mold portion presenting a refractory surface complementary in size, shape and contour to said finned side of said head, a mold portion presenting an uninsulated surface of bare metal complementary in size, shape and contour to said combustion chamber cavity, said uninsulated metal surface comprising a part of a hollow walled element the walls of which are provided with a fluid circulation inlet and outlet passage, said hollow walled element including a plurality of segments generally spaced from each other but yieldably connected together, and yieldable heat resisting means bridging the space between said segments.

JULIUS DUSEVOIR.